

## UNITED STATES PATENT OFFICE.

BY RAMJI D. SAKLATWALLA, OF CRAFTON, PENNSYLVANIA, ASSIGNOR TO VANADIUM CORPORATION OF AMERICA, OF BRIDGEVILLE, PENNSYLVANIA, A CORPORATION OF DELAWARE.

## VANADIUM ALLOY.

No Drawing.

Application filed February 2, 1928. Serial No. 251,465.

This invention relates to a composition of alloy containing vanadium as the major constituent, the remainder being principally iron, and especially to a ferro-vanadium alloy containing over 85% of vanadium.

In the manufacture of vanadium steel in the basic open hearth process, the vanadium is added to the molten steel after it has been tapped into the ladle. If vanadium were 10 added to the steel bath in such a furnace instead of in the ladle, there would be considerable loss of vanadium owing to the oxidizing conditions existing in the furnace. In the acid open hearth or the electric furnace 15 process, vanadium is sometimes added in the furnace, but also some of the alloy, especially material in finely divided state, is added in the ladle. It is well known in steel making practice that the less the total amount of cold 20 material added in the ladle the better and more uniform are the ingots obtained from pouring such steel. The cold material introduced into the ladle absorbs heat in its process of melting and dissolving into the molten steel 25 and consequently reduces the temperature of the ladle, thus running into the danger of pouring the steel into the molds at a lower temperature than that desired for the production of sound ingots.

30 A further deficiency of addition of alloys in the ladle is the fact that whatever impurities are contained in the alloy are retained in the steel, since no purification or oxidation takes place in the ladle. The 35 amount of vanadium metal added to the steel is calculated from the vanadium content of the alloy added; therefore, whatever percentage of other elements, as impurities, are present in the ferro alloy, are introduced and 40 retained in the steel in the same relative ratio to vanadium as they are present in the ferro alloy. The generally used alloys of vanadium at the present time carry approximately 40% vanadium with certain percentages of 45 silicon, carbon, sulphur, phosphorus, etc. It is readily to be seen that, with the same percentages of impurities in the alloy as at present, but with a vanadium content more than twice the present content, the impurities introduced into the steel will be lessened to one-

half the present extent. In the manufacture of alloy steels of very high-grade quality, this is a decided advantage.

By the composition of my invention, I propose to obviate all the above mentioned deficiencies by producing an alloy containing at least 85% vanadium, the balance being mostly iron. An alloy containing this high percentage of vanadium is very readily soluble in molten steel, much more so than the 55 lower percentage alloys, on account of its greater chemical reactivity. Further, since the amount of metalloids, such as silicon, carbon, etc. that are introduced into molten steel per unit of vanadium added are so much less, 60 the diffusion and solution of this alloy is more complete and regular since carbides, silicides, and other such compounds are present only to a very negligible extent. Also, since the bulk of material added per ton of steel is less 65 in this case than in the generally used alloy, there is no difficulty in getting the entire amount of alloy into the ladle before the appearance of any slag from the tap hole.

The alloy of my invention, consisting approximately from 85% to 95% or more vanadium, can be produced in the electric furnace by the use of a suitable reducing agent, such as silicon; however, I prefer to produce same by the reduction of a very high grade 75 of vanadium pentoxide by means of aluminum as reducing agent, according to the well known process of alumino-thermic reduction. An alloy produced by this process from a high-grade oxide has the advantage of not 80 being contaminated with carbon and silicon to an appreciable extent, which would be the case were it produced by reduction by means of silicon in the electric furnace. If care is 85 exercised in the preparation of the vanadium 90 pentoxide, and the reduction material, keeping same free from excessive percentages of impurities, a resulting alloy can be obtained by alumino-thermic reduction containing vanadium and iron alone with negligible percentages of deleterious impurities, and in 95 which the silicon is less than 1.25% and the carbon less than .50%. Such an alloy enables the steelmaker to make his additions without fear of altering the composition of 100

his finished steel in regard to impurities, thus avoiding the possibility of obtaining reject heats of the finished steel.

While I have specifically described the preferred manner of carrying out my process, it will be understood that the process may be otherwise practiced within the scope of the following claims.

I claim:—

1. A ferro-vanadium containing between 10 about 85% to 95% vanadium.

2. A ferro-vanadium containing between about 85% to 95% vanadium, less than 1.25% silicon and less than .50% carbon, the remainder being principally iron.

In testimony whereof I have hereunto set my hand.

BYRAMJI D. SAKLATWALLA.